

## [54] VIBRATORY FORMING

[75] Inventors: **Graham Robert Dawson, Bewdley; Dennis Hugh Sansome, Sutton Coldfield, both of England**

[73] Assignee: **National Research Development Corporation, London, England**

[22] Filed: **Mar. 17, 1972**

[21] Appl. No.: **235,546**

## [30] Foreign Application Priority Data

Mar. 18, 1971 Great Britain ..... 7201/71

[52] U.S. Cl. .... **72/283, 72/56, 72/DIG. 20, 72/285**

[51] Int. Cl. .... **B21d 26/02, B21c 1/24**

[58] Field of Search. .... **72/DIG. 20, 274, 72/283, 285, 56**

## [56] References Cited

## UNITED STATES PATENTS

3,212,312 10/1965 Boyd et al. .... 72/DIG. 20

3,209,573 10/1965 Boyd et al. .... 72/DIG. 20  
2,393,131 1/1946 Vang ..... 72/DIG. 20

Primary Examiner—Charles W. Lanham

Assistant Examiner—M. J. Keenan

Attorney—Cushman, Darby & Cushman

## [57] ABSTRACT

A vibratory forming method, and apparatus, in which material is drawn across a pair of forming tools which are both vibrated. The phase angle between the two vibrations is neither zero nor 180°, but is adjusted to a defined intermediate value to increase the efficiency of the process, especially by minimising the drawing force required. The invention applies particularly to the plug drawing of metal tube.

3 Claims, 14 Drawing Figures



PATENTED JAN 8 1974

3,783,668

SHEET 1 OF 5



PATENTED JAN 8 1974

3,783,668

SHEET 2 OF 5

VARIATION OF OPTIMUM PHASE ANGLE  
WITH VELOCITY RATIO.



Fig. 3.

PATENTED JAN 8 1974

3,783,668

SHEET 3 OF 5

MINIMUM AMPLITUDE RATIO AGAINST  
VELOCITY RATIO FOR OPTIMUM  
PHASE ANGLE.



PATENTED JAN 8 1974

3,783,668

SHEET 4 OF 5

Fig. 5.





Fig. 6.



Fig. 7.



Fig. 8



Fig. 9

## VIBRATORY FORMING

This invention relates to the reduction of metals and other materials by drawing them past at least two tools. In particular it relates to drawing metal rod through a succession of dies, first coarse and then fine, and to drawing tube through the clearance between a female die and a male die, the latter being generally known as a plug. It has already been proposed, in plug drawing, to vibrate both the die and the plug axially while drawing proceeds; see for example U.S. Pat. No. 3,212,312, corresponding to UK No. 1,075,331. However, although such documents refer generally to the possibility of varying the relationship between the vibrations of the plug and those of the die, and have specifically mentioned the possibilities that such vibrations could be in-phase or 180° out-of-phase, they did not suggest how to set about an analysis of this relationship nor of course the optimum values that such an analysis might reveal.

We have now devised and carried out such an analysis. It is summarised later in this specification and leads to the surprising conclusion that optimum performance is in certain cases achieved when the phase angle between plug and die is neither 0° nor 180° but is somewhere between the two, the value depending upon several factors peculiar to the case.

Broadly speaking our invention includes vibratory forming operations using a pair of vibrating tools in which the phase relationship between the tools is substantially the optimum which will be described. Our invention includes apparatus set to achieve such optimum performance.

The invention is formally defined by the claims at the end of this specification and will now be described, by way of example, with reference to the accompanying drawings in which:

FIG. 1 is a diagrammatic side elevation of suitable apparatus,

FIGS. 2a. to 2f. illustrate the relative positions of die and tube at six stages of a cycle of die oscillation,

FIGS. 3 and 4 are graphs showing typical relationships between important parameters discussed in the analysis, and

FIGS. 5 to 9 are graphs in which other parameters from the analysis are each plotted against time.

FIG. 1 shows an input or original metal tube 1 being reduced to a final tube 2, of smaller internal and external diameter, by being drawn through the clearance 3 between a male die or plug 4 and a female die 5. The tube is drawn through this clearance by gripping jaws 6 mounted on a drawing device (not shown) which supplies the drawing force and moves in pace with the drawn tube. Plug 4 is mounted, as is usual, on a plug bar 7. This bar is supported from a plug vibrator 8, which imparts axial vibrations to bar and plug. Female die 5 is connected to a die vibrator 9, which imparts co-axial vibrations to the die, and vibrators 8 and 9 are linked to a control device 10 which controls the relative phase of the two vibrations.

Drawing takes place whenever there is relative movement between tube 1 and the die 5. Using known apparatus the drawing force, i.e., the force required to reduce the tube by pulling it through the die and plug would need to exceed the sum of two other forces. The first of these would be the die force, i.e., the force with which the outer surface of the original tube resists

being pulled and deformed through the die. The second would be the plug force, i.e., the frictional force created by pulling the inner surface of tube 1 over the plug 4. By moving the plug at the same speed as the final tube 2 during drawing, and in the same sense, the plug force disappears and so the drawing force has only to exceed the die force. By moving the plug faster than the tube the plug force actually contributes to the drawing force, so that the drawing force then equals the difference between the die and plug forces, not their sum. Since the maximum reduction in area that can be brought about in the original tube 1 varies as the tensile strength of the final tube 2, it is important to keep the maximum drawing force low and this invention shows 15 a way of doing this. By moving the plug faster than the final tube, the drawing force may be decreased by twice the plug force and still draw at the same rate as before. This can represent a 60 percent gain in machine capacity since the plug force can equal 30 percent of drawing force.

FIG. 2, parts a to f, illustrates the relative motion of final tube 2 and female die 5 during a typical drawing operation. Reference A represents the amplitude of oscillation of the die. Part 2a shows die 5 at the extreme rearward end of its stroke relative to the direction 11 in which the tube is being drawn. At this stage drawing is taking place, that is to say there is such tension in the tube that it is moving through the die from left to right. In part 2b the oscillation of the die has started it moving again towards the right; tension in the tube is still sufficient to cause drawing at the die, but the motion of the die means that the velocity of the tube through the die is less than before, and is diminishing. Part 2c shows the point in time where drawing stops because the relative velocity has dropped to zero. From now until the moment illustrated in part 2f there is no relative movement between die and tube, and thus no draw. Part 2d shows the die at the extreme right hand or forward end of its stroke; since the moment shown in part 2c, the further motion of the die 5 has tended to diminish still further the tension in the final tube 2. Part 2e shows the die on the backward stroke of its oscillation, building up the tension again in the drawn tube, and part 2f illustrates the point in time when the tension has again reached the level necessary to cause drawing. Because of the many variable factors that contribute to the tension in the final tube 2, the positions of the die in parts 2c and 2f are not necessarily the same. Nevertheless, since drawing starts at the position shown in part 2f and continues until a position corresponding to part 2c is next reached, the present invention aims at so relating the vibrations of plug 4 and die 2 that the plug 4 is at least stationary relative to the final tube 2, and preferably has a positive (i.e., rightwards) movement relative to it, for the entire period during which drawing is taking place.

We will now summarise the theoretical considerations that led to the relationships on which this invention is based.

Key to symbols used:

A Die amplitude

b Plug Plug amplitude

n B/A

w angular frequency

$\pi/2 + \theta$  phase lead of plug over die

V Drawing speed

x displacement

$\delta$  relative movement of ends of tube during period of elastic loading and offloading  
 $F$  non-oscillatory drawing force  
 $\Delta F$  non-oscillatory plug force  
 $f$  oscillatory drawing force  
 $f_p$  oscillatory plug force

Suffixes

1. Die
2. Tub at die
3. Other end of tube (i.e., at gripping jaws 6)
4. Plug

The following assumptions have also been made:

1. The magnitude of the plug force is unaltered by its periodic reversal ( $f_p = \pm \Delta F$ )
2. The deformation pattern is unaltered by the reversal of plug forces ( $f_{max} = F - 2\Delta F$ )
3. Inertia forces in the tube are negligible
4. The drawing velocity is constant (no periodic component due to the cyclic forces imposed)
5. The drawing force exerted by jaws 6 is constant.

At time  $t = 0$  let the die be at its most backward position and let the plug have a phase lead of  $\theta/2 + \theta$  over the die. Furthermore assume drawing to be occurring.

Thus:

$$x_1 = A \cos \omega t \quad (1)$$

$$x_4 = B \sin (\omega t + \theta) \quad (2)$$

and until drawing stops  $x_2 = x_3 = V$ , since the drawing force is constant. Drawing will stop when the relative velocity of tube and die reaches zero, at  $t + t_1$ .

i.e., when  $x_2 - x_1 = 0$

i.e.,  $v - Aw \sin \omega t_1 = 0$

Thus drawing stops at  $t = t_1$  where

$$\omega t_1 = \sin^{-1} V/Aw = \phi \text{ say.} \quad (3)$$

From this time, since drawing has stopped, the tube at the die will follow the die, whilst the other end will have a constant velocity  $V$ . This will result in a period of elastic offloading and loading. During this period:

$$\delta = |x_3 - x_2|_{t_1}^t = \dot{x} = V, \quad \int_{t_1}^t (\dot{x}_3 - \dot{x}_2) dt$$

where  $x_3 = V$ , and

$$x_2 = x_1 = Aw \sin \omega t.$$

Thus  $\delta = A \cos \omega t_1 - A \cos \omega t + V(t_1 - t)$ .

Drawing will restart when the drawing force felt at the die returns to that exerted at 6 (see FIG. 5).  $\delta$  becomes zero at  $t = t_2$ , where from above:

$$A \cos \omega t_2 + Vt_2 = A \cos \omega t_1 + Vt_1.$$

Combining with (3), this gives:

$$A \cos \omega t_2 + Vt_2 = A \cos \phi + V\phi/w \quad (4)$$

During the drawing period determined above, the velocity of the plug relative to the tube must be zero or in the positive direction throughout, if the forces are to be reduced. This period of reversed friction has a maximum of  $2\pi/w$ , for zero drawing speed, and reduces with increasing drawing speed. The system is optimised when the period of reversed friction is equal in duration to the drawing period and is synchronised with it, since no further increase in speed may be tolerated without reverting to the conventional drawing force. This corresponds to friction reversing at  $t = t_1$  and  $t_2$ .

Thus:

$$\text{at } t = t_1,$$

$$\dot{x}_2 = \dot{x}_4, \text{ and}$$

$$V = Bw \cos (\omega t_1 + \theta).$$

$$\therefore \cos (\omega t_1 + \theta) = V/nAw = \sin \phi/n$$

(from (3))

5

$$\therefore n = \sin \phi / \cos (\phi + \theta) \quad (5)$$

and at  $t = t_2$ ,

$$\dot{x}_2 = \dot{x}_4, \text{ and}$$

$$\cos (\omega t_2 + \theta) = \sin \phi/n \text{ as above.}$$

$$\therefore \omega t_2 + \theta = \cos^{-1} \sin \phi/n \text{ or } 2\pi - \cos^{-1} \sin \phi/n$$

$$\text{where } \cos^{-1} \sin \phi/n \leq \pi.$$

Since  $\omega t_2$  does not equal  $\omega t_1$  the second solution is correct.

$$\omega t_2 = 2\pi - \theta - \cos^{-1} \sin \phi/n \quad (6)$$

Substituting for  $n$  from (5)

$$\omega t_2 = 2\pi - 2\theta - \phi \quad (7)$$

Substituting in (4) to obtain  $\theta$  in terms of  $\phi A \cos (2\phi + \theta) + V/w (2\pi - 2\theta - \phi) = A \cos \phi + V\phi/w$  which simplifies to:

$$\sin \theta \cot \phi + \cos \theta = \pi - \theta - \phi / \sin \theta \quad (8)$$

25 Equation (8) expresses the optimum phase angle for a give value of  $\phi$ . This was solved by plotting the right hand side against the left for a range of values of  $\phi$ , each with a range of values of  $\theta$  and interpolating the correct  $\theta$ . FIG. 3 gives the variation of optimum phase angle with velocity ratio,  $\sin \phi$ . FIG. 4 gives the variation of the corresponding value of amplitude ratio,  $n$ , with velocity ratio,  $\sin \phi$ . This expresses the minimum value of plug amplitude necessary for friction reversal or at least elimination to occur throughout the drawing period, when the optimum phase angle is used.

30 FIGS. 5 - 9 illustrate several realtionships referred to in the above analysis.

Another important quantity is the velocity ratio,  $\sin \phi$ , that is to say the ratio between the drawing speed  $V$  and the angular velocity of the oscillation of female die 5. Now for there to be reversed motion, or in the limiting case no relative motion at all between plug and die throughout the drawing period, the drawing interval must not exceed one half cycle or  $\pi$ .

35 45 Now friction reverses when  $t = t_1$ , i.e., where  $\omega t_1 = \phi = \sin^{-1} V/Aw$

Friction also reverses when  $t = t_2$  where  $A \cos \phi + V\phi/w =$

$$A \cos \omega t_2 + Vt_2.$$

50 55 In the critical condition  $\omega t_2 = \pi + \omega t_1 = \pi + \phi$ .

$$\therefore A \cos \phi \cdot \max + V\phi \cdot \max / w = A \cos(\phi + \pi) +$$

$$V/w(\phi \cdot \max + \pi)$$

$$\therefore 2A \cos \phi \cdot \max = V\pi/w$$

$$\therefore \cos \phi \cdot \max = \pi/2 \sin \phi \cdot \max$$

$$\therefore \tan \phi \cdot \max = 2/\pi$$

$$\therefore \sin \phi \cdot \max = 0.5370 = (V/Aw) \cdot \max \quad (9)$$

This in effect limits the process at present to drawing speeds of up to 500 feet per minute, because of the limit to the oscillatory velocity that can be obtained with current vibrators conveniently available.

60 The above analysis gives data to optimise the process. The main factors are:

(1) For a velocity ratio ( $V/Aw$ ) in excess of 0.537 the process is ineffective.

(2) For a velocity ratio less than that there is an optimum phase angle between die and plug oscillations.

- (3) At this velocity ratio, and with the optimum phase angle, there is a minimum amplitude ratio ( $n$ ) below which the process is ineffective.  
 (4) At the optimum phase angle, drawing velocity is maximised, all else being held constant, or the plug amplitude is minimised, all else being held constant.

If, in an actual process the phase angle and amplitude ratio are set corresponding to a high value of velocity ratio,  $\sin\phi$ , there remains the question: is the process effective for lower values of  $\phi$ , which correspond to low speeds encountered when drawing is initiated. Now for lower values of  $\phi$  the optimum phase angle  $\theta$  is reduced. Thus if  $\theta$  is held constant, optimised for a high value of  $\phi$ , and  $\phi$  is reduced, then the drawing period occurs later, and the reversed friction period remains unmoved. If  $n$ , and hence the plug amplitude, is reduced, then the instant of friction reversal will coincide first with the instant when drawing stops. This condition is said to be critical since any further reduction of  $n$  will result in drawing at a higher load.

Now:

$$x_1 = -A \cos \omega t$$

$$x_4 = B \sin (\omega t + \theta)$$

as before, but  $\theta = \text{constant}$ .

Drawing stops when:

$$Aw \sin \omega t_1 = V$$

$$\omega t_1 = \sin^{-1} V/Aw = \phi \quad \text{The critical value of } n \text{ is given by}$$

$$Bw \cos (\omega t_1 + \theta) = V$$

$$n = \sin\phi/\cos(\phi + \theta)$$

This gives the critical value for  $n$  for both the high, optimised value of  $\phi$ , and for those values below. The process is said to be effective if  $n$  continually reduces with  $\phi$ , so that the critical value at the optimised condition is always in excess of that corresponding to lower values of  $\phi$ .

This is so if  $dn/d\phi > 0$  for the whole range.

$$\text{Now } dn/d\phi = \cos(\phi + \theta) \cos\phi + \sin\phi \sin(\phi + \theta)/\cos^2(\phi + \theta) = \cos\theta/\cos^2(\phi + \theta)$$

$$\therefore dn/d\phi > 0 \text{ if } -\pi/2 > \theta > \pi/2$$

But from FIG. 4.0  $0 > \theta > 58^\circ 30'$  and thus the process is effective for speeds up to the optimum condition.

Although described with relation to apparatus and a process for the plug drawing of tube, the invention is applicable also to other apparatus and processes in which material is passed through several tools. By oscillating these tools at the correct phase angle a reduction in total drawing force can be achieved by operating one tool to cause intermittent deformation and operating the other with such phase that frictional constraint by that tool upon the deformation either disappears or is reversed. This can apply to many known processes in which deformation is associated with two tools, e.g., deep drawing. In such applications, of course, the limiting values for velocity ratio, amplitude ratio etc. may be different but may be determined by similar analysis.

Extra effects will also have to be taken into consideration if the second tool exerts not only the frictional constraint of the parallel-sided plug described in this specification. For instance the second tool could also deform to some extent.

It should also be noted that the vital related vibrations to which this invention applies are those at the die and at the plug. It is normally not difficult to position the die vibrator (9) close to the die itself (5) so that the vibrations of the vibrator are very similar in time and all other respects to those at the die itself. However, vibrations can only be transmitted to the plug through the plug bar 7. This bar, which may be quite long, will ensure that the vibrations of the plug do not correspond with those of vibrator 8. Vibrator 8 must therefore be set so that not its own vibrations, but those at the other end of the bar, are correct. The difference will tend to be the greater the lower the frequency of the vibrations, e.g., if they are in the sonic range.

It is also unnecessary, although often simpler for the purposes of analysis, that the vibrations should be sinusoidal. They may be of other types, provided the phase angle between die and plug can be practically ascertained.

25 We claim:

1. A method for vibratory forming in which material is drawn across at least one pair of tools, in which each tool of the pair is vibrated axially while drawing proceeds, and in which the phase angle between the two vibrations is such that while the material is drawing relative to one of the pair of tools the other tool has a velocity no lower than zero, relative to the material, in the direction of drawing.

2. A method for vibratory forming according to claim 1 in which a tube is drawn through a clearance between said pair of tools, comprising a female die and a male plug, and in which the equation:

$$\sin \theta \cot \phi + \cos \theta = -\theta - \phi/\sin \theta$$

is satisfied, where the phase lead of the plug over the die is  $\pi/2 + \theta$  and where  $\phi = 2\sin^{-1} V/Aw$ ,  $V$  being the drawing speed,  $A$  the amplitude of the vibrations of the die and  $w$  their angular frequency.

3. Plug drawing apparatus for drawing metal tube comprising a female die and a male plug defining an annular orifice through which the tube is drawn axially, first means to vibrate both die and plug in a direction parallel to said axis, and second, adjustable means controlling the relationship between the vibrations of said die and said plug, said second means being so set that the equation:

$$\sin \theta \cot \phi + \cos \theta = -\theta - \phi/\sin \theta,$$

is satisfied where  $\pi/2 + \theta$  is the phase lead of the vibrations of the plug over those of the die and where  $\phi = \sin^{-1} V/Aw$ ,  $V$  being the drawing speed,  $A$  the amplitude of the vibrations of the die and  $w$  their angular frequency.

\* \* \* \* \*